# EUROPEAN PATENT APPLICATION

(11) **EP 4 603 608 A1**
(43) Date of publication of application: **20.08.2025**
(21) Application number: 23913865.4
(22) Date of filing: 26.12.2023
(51) Int. Cl.: C22B 1/24, C22B 1/243

(54) **PROCESS FOR PRODUCING IRON ORE AGGLOMERATE FOR USE IN DIRECT REDUCTION REACTORS, AND AGGLOMERATE PRODUCT**

(30) Priority: 06.01.2023 BR 102023000265; 06.12.2023 BR 102023025626
(71) Applicant: Vale S.A., 22250-145 Botafogo, Rio de Janeiro, RJ (BR)
(72) Inventor: DE RESENDE, Valdirene Gonzaga, 30492-020 Belo Horizonte, MG (BR); DUTRA, Flávio de Castro, 36492-335 Ouro Branco, MG (BR); PARREIRA, Fabricio Vilela, 30320-060 Belo Horizonte, MG (BR); PIMENTA, Felipe Viana, 30310-730 Belo Horizonte, MG (BR)
(74) Representative: Grünecker Patent- und Rechtsanwälte PartG mbB
(86) International application number: PCT/BR2023/050498
(87) International publication number: WO 2024/145703

(57) **Abstract**

The process for producing iron ore agglomerates for use in direct reduction furnaces involves dispersing nanomaterial in a binder, combining it with iron ore fines and/or steelmaking by-products along with additives, adjusting moisture, carrying out agglomeration, curing the agglomerate, and applying a surface coating to mitigate the sticking effect within direct reduction furnaces.

## Description

### FIELD OF THE INVENTION

The present invention pertains to the field of mining-metallurgical technologies and refers to a process of iron ore agglomerate production for application in direct reduction (DR) reactors, thereby replacing the pellets and lumps traditionally used.

### BACKGROUND OF THE INVENTION

Direct reduction reactors are characterized by reducing iron ore to metallic iron without melting the burden in the reactor. The metallic product obtained in the solid phase is called sponge iron (a.k.a. DRI - Direct Reduced Iron), which can be hot briquetted, thereby obtaining the Hot Briquetted Iron (HBI).

The direct reduction process is an alternative to using the blast furnace for manufacturing an intermediate product with the same basic functions as pig iron produced by the blast furnace. Both intermediate products (pig iron and sponge iron) are intended for use in the steelworks for the production of steel, with sponge iron being used in electric furnaces. The best-known direct reduction processes are Midrex, HyL (Hayata y Lamina), Armco, H. Iron, SL-RN, and Purofer.

In order to ensure an optimized performance of direct reduction reactors, as well as a high-quality final product (sponge iron), the iron ore agglomerate to be fed needs to have specific physical-chemical-metallurgical characteristics.

The current state of the art provides for some ore agglomeration technologies for application in reduction furnaces. However, none of such technologies results in agglomerates with specific metallurgical characteristics for optimized performance in a direct reduction reactor, as provided by the present invention.

Vale S.A.'s patent BR102019023195-5 describes an agglomerate of iron ore fines to replace metallic burdens in blast furnaces, unlike the present invention, which produces agglomerates with specific characteristics to feed direct reduction reactors, such as Midrex and HyL. Furthermore, patent BR102019023195-5 uses fluxes and inputs other than those from the present invention. Moreover, said patent does not have coating application steps, as required in the present invention.

Patent BR112014005488-6, also in the name of Vale S.A., describes a process for obtaining agglomerates that, in several aspects, differs from the present invention, including (i) raw materials employed, (ii) lack of a coating stage, (iii) application to agglomerates obtained by pelletizing technology (e.g., mini pellets), and (iv) the product subject to the patent does not have physical and chemical requirements for application in the direct reduction process.

Patent application BR102022006033-9, also in the name of Vale S.A., describes a process for obtaining agglomerates that differs from the present invention in terms of (i) the raw materials employed, (ii) the use of microwaves for reduction, (iii) the use of biomass as a reducer, and other differences. Document BR102022006033-9 describes a process for obtaining reduced material through microwave technology and biomass. The resulting pre-reduced agglomerate (metallic Fe >60%) is only an intermediate step for future application in different reactors.

The master's thesis entitled *"*Desenvolvimento de briquetes autorredutores com agente de recobrimento" (Development of self-reducing briquettes with coating agent), published in 2019 by Kleiton Gonçalves Lovati, describes a process for obtaining self-reducing briquettes that use coating agents such as dolomitic limestone, bentonite, serpentinite, and steelmaking slag. The present invention differs from this document as it is a different product and cannot be considered a self-reducing briquette. Self-reducing briquettes are composed of iron ore and a significant amount of carbonaceous material so as to provide them with their self-reducing characteristic. They are specifically used in Reduction and Fusion technologies (e.g., Corex, Finex, Hismelt, Tecnored, Oxicup), unlike the present invention, whose focus is on Direct Reduction technologies (e.g., Midrex, HyL, Fastmet, Jindal, etc.).

The master's thesis entitled *"*Desenvolvimento de metodologic para avaliação à tendência à reoxidação de pelotas de minério de ferro reduzidas em processo de redução direta à g6s" (Development of a methodology to evaluate the reoxidation tendency of iron ore pellets reduced through direct gas reduction process), published by Renata Gonçalves Penna in 2010, describes the effect of degradation of iron ore pellets in a direct reduction process. Distinguishing itself from the present invention, this document pertains to a dissimilar agglomeration process. Specifically, the document focuses on pellets generated through a hot agglomeration process (> 1300 °C), whereas the present invention deals with cold agglomeration carried out at a temperature of approximately 250 °C.

In direct reduction agglomerates, the iron content has to be higher (> 60%) and the deleterious content (Na₂O, SiO₂, and Al₂O₃) lower (< 10%) when compared to the blast furnace process. Furthermore, it is essential that agglomerates for direct reduction need to have low disintegration and high metallization content (> 90%) when compared to blast furnace products.

The present invention relates to a process for producing cold iron ore agglomerate for use in direct reduction (DR) reactors, which presents the following benefits when compared to processes known in the prior art:
1. Agglomerate porosity control via incorporation of organic additives and curing at slightly higher temperatures (burning of added organic materials);
2. Compaction degree control via reduction of compaction pressure and bulk density of the agglomerate;
3. Application of necessarily richer feeds (ore feed with higher iron content);
4. Application of one or a combination of binders;
5. Standard-sized agglomerate, which influences the properties of the final product;
6. Agglomerate with high physical resistance to handling and transportation over long distances, including resistance to weathering;
7. Agglomerate that provides low generation of fines in reduction reactors and a high degree of metallization;
8. Reduction in CO₂ emissions, as curing takes place at room temperature or low temperature.

The porosity for this type of agglomerate is critical for its subsequent application in direct reduction reactors. To this end, control of porosity and degree of compaction are the differentiating and essential factors that can promote the necessary properties of the product for its use in direct reduction reactors.

Porosity control, for example, allows gases to enter and leave the internal structure of the agglomerate during the direct reduction process without compromising its physical quality, that is, disintegrating. Otherwise, the product's resistance is highly impacted, and the product fails to meet the minimum performance standards essential for the process.

Agglomerate compaction can be controlled by adjustments to process conditions, by improving the agglomerate finish and using additives (chemical or mineral) to ensure optimal porosity.

Therefore, the present invention greatly differs from the documents known in the state of the art since the importance of porosity for this direct reduction product was verified in bench-scale tests, as well as in basket tests in direct reduction process in some customers.

Regarding the production supplies, it is important to note that the potential utilization of a blend of various binders aims, among other objectives, to diminish the presence of deleterious substances (Na₂O, SiO₂, and Al₂O₃) in the agglomerated product.

### OBJECTIVE OF THE INVENTION

The present invention's general objective is to provide a new production process for iron ore agglomerate with high metallurgical performance to replace lumps and pellets in direct reduction reactors. The main characteristics of the resulting agglomerate are high physical resistance, low generation of fines, and a high degree of metallization during operation in direct reduction reactors.

Another objective of the present invention is to provide a more sustainable process for the reduction of CO₂ emissions in the mining-metallurgical production chain.

### SUMMARY OF THE INVENTION

The present invention, in its preferred embodiment, discloses a production process for iron ore agglomerate to replace lumps and pellets in direct reduction furnaces comprising the following steps:
a) Disperse 0.05-2% per weight of nanomaterial in the binder in order to obtain a "binding mixture";
b) Mix 1-10% of the binding mixture from step a) with 70-99% iron ore fines and/or steelmaking by-products, 0-5% chemical and/or mineral additives with properties to promote plasticity and/or improve the agglomerate's porosity;
c) Adjust the moisture to obtain 0-25% per weight of water in the mixture;
d) Perform the agglomeration process via briquetting or extrusion;
e) Cure the agglomerate;
f) Apply coating at the surface of the agglomerate to reduce the sticking effect in DR reactors;

### BRIEF DESCRIPTION OF THE DRAWINGS

The present invention is described in detail based on the respective figures:
Figure 1 illustrates a simplified block diagram of the agglomerate production process for use in direct reduction reactors, according to the present invention.
Figure 2 presents a comparison showing the evolution of the disintegration results of the resulting agglomerates.
Figure 3 shows an image of the agglomerates resulting from the present invention's process after applying the coating used to mitigate the sticking effect.
Figure 4 shows an image of the agglomerates (DRI) obtained after a basket test in a direct reduction reactor on an industrial scale.
Figure 5 shows a graph containing agglomerate metallization and carburization data (DRI) from the various briquette samples subjected to basket tests in Midrex and HyL reactors.
Figure 6 shows a graph containing data of disintegration under reduction of agglomerates (DRI) obtained with the various briquette samples subjected to basket tests in Midrex and HyL reactors.

### DETAILED DESCRIPTION OF THE INVENTION

Although the present invention may be susceptible to different embodiments, the preferred embodiments are depicted in the figures and elucidated in the subsequent detailed discussion, where it should be understood that this description serves as an illustration of the principles of the invention and is not meant to constrain the present invention solely to what has been depicted and described here.

The matter required in the present invention will be expanded upon hereinafter, by way of example and not limitation, since the materials and methods disclosed herein may comprise different details and procedures without departing from the scope of the invention. Unless otherwise indicated, all parts and percentages disclosed below are per weight.

The main approach of this invention is related to a production process for iron ore agglomerate to replace lumps and pellets in direct reduction furnaces comprising the following steps:
a) Disperse 0.05-2% per weight of nanomaterial in the binder in order to obtain a "binding mixture";
b) Mix 1-10% of the binding mixture from step a) with 70-99% iron ore fines and/or steelmaking by-products, 0-5% chemical and/or mineral additives with properties to promote plasticity and/or improve the agglomerate's porosity;
c) Adjust the moisture to obtain 0-25% per weight of water in the mixture;
d) Perform the agglomeration process via briquetting or extrusion;
e) Cure the agglomerate;
f) Apply coating at the surface of the agglomerate to reduce the sticking effect in DR.

The agglomerate production process, represented by the block diagram in Figure 1, preferably begins with the dispersion of the nanomaterial in the binder(s) under mechanical stirring at a dosage of 0.05 to 2% per weight in relation to the amount of binder used in the mixture. The nanomaterials used in step a) can be carbon nanotube, exfoliated graphite, functionalized microsilicate, tubular nanosilica, tubular halloysite, carbon nanofiber, and graphene, among others.

The binders used in step a) may consist of sodium silicate, vegetable tar, pitch, starch, phenolic resins, and molasses, among others. Such binders, used to link particles by adhesion and/or chemical interaction, can be used individually or combined to obtain better resistance of the agglomerated product.

Step b) of the process of the present invention consists of adding 1 to 10% of the binder mixture obtained in step a) to 70 to 99% per weight of iron ore fines and/or steel co-products, and 0 to 5% per weight of chemical and/or mineral additives and, then, mixing in an intensive mixer for no more than 4 minutes. The additives used as plasticizing agents consist of bentonite, pitch, tar, starch, and hydrated lime and have the property of increasing plastic conformation during the subsequent agglomeration step. Some porosity-forming substances are also used as additives, such as pitch, tar, phenolic resins, glucose, starch, molasses, glycerin, CMC (carboxy methyl cellulose), and biomass, which promote greater porosity in the agglomerate after curing.

The iron ore fines and steelmaking by-products used in step b) of the present invention's process preferably have Feₜₒₜₐₗ contents > 60%, SiO₂ < 5%, Al₂O₃ < 2%, granulometry 98% < 6 mm, and maximum humidity of 25%. The steelmaking by-products used may consist of pellet fines, DRI (Direct Reduced Iron) fines, sludge, and scale, among others. The quality of such by-products may vary depending on the plant. Thus, their use as raw material is subject to compliance with the grades previously mentioned and through prior laboratory tests.

Step c) of this process consists of adjusting the humidity of the mixture by adding water to obtain the optimal moisture of 0 to 25%, as desired for the agglomeration step.

Step d) of the present invention refers to the agglomeration process that can be carried out by means of briquetting or extrusion.

For agglomeration via extrusion, the optimum moisture should be in the range of 8-25%. In addition to the incorporation of binders and additives, the strength and porosity of the green agglomerate are modulated in the production process by regulating the negative pressure within equipment known as extruders. The resulting extrudates are cylindrical rods of size 5-50 mm in diameter and 50-200 mm in length.

For briquetting agglomeration, the mixture should preferably contain between 1-7% moisture. The briquetting process takes place in a roller press with suitable cavities to obtain briquettes in pillow geometry measuring 15-50 mm x 10-40 mm x 5-25 mm. This geometry and adequate control of these dimensions, associated with the raw materials and process conditions used, result in agglomerates with greater mechanical resistance that generate excellent performance results.

In the briquetting process, it is crucial to regulate the pressure and speed of the rollers, control the distance between rollers (maintaining a minimal gap to prevent the formation of open briquettes and/or those with burrs), and oversee the feeding rate. This is done to achieve a briquette with a bulk density below 3.8 g/cm³ and a compaction degree around or less than 50%, aligning with the desired metallurgical properties.

The pressure and speed of the rollers are controlled by changing the amperage of the briquetting machine, with each machine having a different type of adjustment. It is not possible to define pre-determined amperage ranges, as this can vary greatly depending on the type, brand, and capacity of the briquetting machine. Therefore, a control that is best applied and can be replicated for different machines is through the calculation of linear force, whose recommended value is 15 to 30 KN/cm. The higher the amperage, the greater the force of particle approximation and, consequently, the greater the compaction (packing and bulk density) and the lower the porosity. However, an optimum point between compaction, bulk density, porosity, and the physical quality of the agglomerate is required.

Step e) of the present production process comprises curing the agglomerate, which can be done through gas furnaces, electric, infrared, electromagnetic furnaces or at room temperature. The temperature conditions and curing time in the different types of furnaces will be determined by the type of binder or mixture of binders used. If the binder is pure sodium silicate, 10 to 30 minutes at 100 to 550 ºC is recommended for electric, infrared, or gas furnaces. For microwave-based electromagnetic furnaces, the time would be 2 to 15 min. For curing at room temperature, time adds up to 15 days.

In step f), an additional layer of chemical or mineral agent is applied through methods such as immersion, spray, or alternative technologies, aiming to minimize the sticking of agglomerates within the direct reduction reactors. These additives can be bauxite, bentonite, serpentinite, cement, magnesium hydroxide, limestone, and combinations thereof. The coating agent dosage per ton of agglomerate varies between 1 and 10 kg. The coating is disposed in suspension in water for application.

The iron ore agglomerate produced via the present invention has physical, chemical, and metallurgical attributes that allow it to substitute pellets and lumps in direct reduction furnaces, thus resulting in enhanced efficiency and productivity within the metallurgical chain. The characteristics of the final agglomerate are:
- High iron content (Fe > 60%)
- Low deleterious content (Na₂O, SiO₂, and Al₂O₃ < 5%)
- Low disintegration value (< 10%, reaching values < 5%)
- High metallization content (> 90%, reaching values of 99.5%)

The exceptional performance of the agglomerates derived from the present invention within direct reduction reactors is attributable solely to three critical factors meticulously regulated throughout the process:
- Compaction degree < 50%
- Bulk density < 3.8 g/cm³
- Porosity > 40%, with a network of connected pores

The porosity for this type of agglomerate is critical for its subsequent application in direct reduction reactors. Porosity control, for example, allows gases to enter and leave the internal structure of the agglomerate during the direct reduction process without compromising its physical quality. Otherwise, the product's resistance during reduction is highly impacted, and the product will not have the minimum performance required in the process, thus generating fines through disintegration, which is detrimental to the process in direct reduction reactors.

Figure 2 presents a comparison showing the evolution of the disintegration results obtained throughout the research and development (R&D) process aiming the optimization of the present invention. Figure 2A shows agglomerates resulting from state-of-art processes, showing a high disintegration value in the order of 40 to 65%. Figure 2B shows the first evolution from R&D processes, with disintegration values between 20 and 30%. Figure 2C shows agglomerates resulting from the process described in the present invention, whose disintegration value is below 10%.

The compaction degree of the particles directly influences the level of disintegration of the agglomerates in direct reduction reactors, in addition to improving the degree of metallization. Less dense agglomerates have greater porosity, allowing gases to enter and exit more homogeneously (less abruptly) during the metallurgical operation within a direct reduction reactor, as previously mentioned.

The present invention allows optimal parameters of compaction degree and porosity to be achieved through adjustments in agglomeration conditions, improvement of the agglomerate finish and use of additives (chemical or mineral) to improve porosity.

### EXAMPLE

Agglomerates of iron ore fines for specific use in direct reduction reactors were produced according to the process described by the present invention.

A total of 96% per weight of pellet feed with Fe content = 68.5% and particle size < 0.15 mm were used as iron ore fines. Sodium silicate and nanomaterial were used as binders. The additives used were starch and hydrated lime. The agglomeration process of choice was briquetting, and pillow-shaped briquettes were produced in the following dimensions: 25 x 20 x 15 mm.

The amperage used in the briquetting machine varied between 30 and 40 Å, corresponding to a linear force in the order of 15.7 to 29.4 KN/cm. The briquettes were cured in a gas furnace for 30 min, in a temperature range of 250 - 350 °C. After curing, the briquettes underwent the coating stage through sprayed cement.

The resulting briquettes, as shown in Figure 3, were subjected to chemicalphysical-metallurgical tests in order to attest to the quality of the final agglomerate obtained. The chemical and physical quality results for several briquette samples are shown in Table 1 below:

| **Parameters** | **Resulting values** |
|---|---|
| Fe (%) | 65.1- 67.5 |
| SiO₂ + Al₂O₃ (%) | 1.9-4.7 |
| LOI (%) | 0.2 - 2.3 |
| Bulk density (g/cm³) | 3.1- 3.7 |
| Shatter JIS M 8711 % + 10.0mm | 95 - 99 |
| Tumble, ISO 3271 % + 6.3 mm | 66 - 90 |
| Abrasion, ISO 3271 % - 0.5mm | 10-28 |
| Cold compression strength daN/briquette | 180 - 630 |
| Metallization (%) | 91.2 - 99.5 |
| Disintegration - 3.36 mm (%) | < 10 |
| Carbon (%) | 0.9 - 4.4 |

Figure 4 shows the image of the DRI agglomerates resulting from basket tests conducted in Midrex and HyL industrial reactors. Quality data for these DRI agglomerates, including metallization and carburization (Figure 5) and disintegration under reduction (Figure 6), are shown.

Therefore, while only specific embodiments of the present invention have been illustrated, it should be recognized that a person skilled in the art can make various omissions, substitutions, and modifications without deviating from the essence and extent of the present invention. The described embodiments should be considered in all respects only as illustrative and not restrictive.

It is expressly provided that all combinations of elements that perform the same function in substantially the same way to achieve the same results are within the scope of the invention. Substitutions of elements from one described embodiment to another are also fully intended and contemplated.

## Claims

1. Process for production of iron ore agglomerate for use in direct reduction reactors **characterized by** the following steps:
a) Disperse 0.05-2% per weight of nanomaterial in the binder in order to obtain a binding mixture;
b) Mix 1-10% of the binding mixture from step a) with 70-99% iron ore fines and/or steelmaking by-products and 0-5% additives in an intensive mixer;
c) Adjust the moisture to obtain 0-25% per weight of water in the mixture;
d) Perform the agglomeration process via briquetting or extrusion;
e) Cure the agglomerate;
f) Apply coating at the surface of the agglomerate to reduce the sticking effect in DR furnaces.

2. Process, according to claim 1, wherein the nanomaterial used in step a) is selected from the group consisting of carbon nanotube, exfoliated graphite, functionalized microsilicate, tubular nanosilica, tubular halloysite, carbon nanofiber, and graphene.

3. Process, according to claim 1, wherein the binder used in step a) is selected from the group consisting of sodium silicate, vegetable tar, pitch, starch, phenolic resins, and molasses.

4. Process, according to claim 1, wherein the iron ore fines and steelmaking by-products employed in step b) have Feₜₒₜₐₗ contents > 60%, SiO₂ < 5%, Al₂O₃ < 2%, and granulometry 98 % < 6 mm.

5. Process, according to claim 1, wherein the additives used in step b) are selected from the group consisting of bentonite, pitch, tar, hydrated lime, phenolic resins, glucose, starch, molasses, glycerin, CMC (carboxy methyl cellulose), and biomass.

6. Process, according to claim 1, wherein the mixing in step b) is carried out in an intensive mixer for no more than 4 minutes.

7. Process, according to claim 1, wherein the agglomeration in step d) is performed in extruders producing extrudates in the shape of cylindrical rods of size 5-50 mm in diameter and 50-200 mm in length.

8. Process, according to claim 1, wherein the agglomeration in step d) is performed in a roller press producing briquettes in pillow format with dimensions 15-50 mm x 10-40 mm x 5-25 mm.

9. Process, according to claim 1, wherein the agglomeration in step d) is performed in a roller press producing briquettes with a packing degree < 50%, bulk density < 3.8 g/cm³, and porosity > 40%, with connected pores.

10. Process, according to claim 1, wherein the agglomeration in step d) is performed in a briquetting machine controlling the linear force in the range of 15 to 30 KN/cm.

11. Process, according to claim 1, wherein curing in step e) can be carried out in gas, electric, infrared, electromagnetic furnaces or at room temperature.

12. Process, according to claim 11, wherein curing in gas, electric, or infrared furnaces is carried out at a temperature of 100 to 550 °C for 10 to 30 minutes.

13. Process, according to claim 11, wherein curing in electromagnetic furnaces is carried out for 2 to 15 minutes.

14. Process, according to claim 11, wherein curing at room temperature is carried out for up to 15 days.

15. Process, according to claim 1, wherein the application of coating agent in step f) is done by immersion or spraying a chemical or mineral additive with surface covering properties selected from the group consisting of bauxite, bentonite, serpentinites, cement, magnesium hydroxide, limestone, and combinations thereof.

16. Process, according to claim 1, wherein the dosage of coating agent is 1 to 10 kg per ton of agglomerate in step f).

17. Iron ore agglomerate produced from the process described in claims 1 to 16, **characterized by** having optimal physical, chemical, and metallurgical properties to replace pellets and lumps in direct reduction furnaces, namely Fe > 60%, deleterious content (Na₂O, SiO₂, and Al₂O₃) < 10%, disintegration < 10%, metallization content > 90%, degree of packing < 50%, bulk density < 3.8 g/cm³, and porosity > 40%, with connected pores.

18. Agglomerate, according to claim 17, **characterized by** having Fe content in the range of 65.1 to 67.5%, deleterious content (Na₂O, SiO₂, and Al₂O₃) < 5%, disintegration < 5%, and metallization content in the range of 91.2 - 99.5%.
